

## UNITED STATES PATENT OFFICE

WILHELM SAILER, OF SCHWAAN, GERMANY, ASSIGNOR TO THE MEAD RESEARCH ENGINEERING COMPANY, OF DAYTON, OHIO

## TREATMENT OF ANIMAL SKINS AND PELTS

No Drawing. Application filed December 12, 1929, Serial No. 413,686, and in Germany April 25, 1929.

The present invention relates to the treatment of animal skins and pelts.

The employment for tanning purposes, of sulphite cellulose liquor and lignin sulphonic acid and of their chlorination and esterification products is known.

These processes are only partially satisfactory however. I have found by experiments that, in working up skins and pelts to good quality leathers novel tanning effects can be obtained if, for tanning purposes, use is made of spent liquor from the manufacture of sulphite cellulose, or lignin sulphonic acid, which has been treated with hydrogen peroxide and has subsequently been acted upon by chlorine or bromine, or both halogens together.

Instead of hydrogen peroxide, corresponding solutions of compounds capable of liberating oxygen, such as perborates, persulphates and the like, may be used.

In the place of spent sulphite cellulose liquor or lignin sulphonic acid, use may be made of natural tanning agents, or mixtures of any of these substances with or without further admixture of phenols, cresols or similar compounds of the aromatic series, for instance quinones or such naphthol and anthracene compounds which contain one or more OH groups, such as polyphenols and the like, these compounds or their mixtures being also subjected to treatment with hydrogen, "persalts" or the like and halogens.

Instead of spent sulphite cellulose liquors, mixtures of such liquors and natural tanning substances may be used. It is also possible to use natural tanning substances alone. To these substances hydrogen peroxide or solutions of compounds capable of liberating oxygen may be used and simultaneously or subsequently chlorine or bromine or both halogens together may be allowed to act upon the mixture.

It is further possible to use, instead of natural tanning substances, mixtures of same with the above named phenols, cresols or similar compounds of the aromatic series.

If reaction products of this kind are diluted with water and animal skins without hair, hides or pelts are tanned therewith, a very

novel effect not hitherto known and of pronounced technical importance is obtained.

The depilated skins and the like, previously treated in this way, can be worked up in the shortest possible time to a leather, which 55 possesses the advantages of a leather which has been pittanned for months, if they are subsequently finishtanned in a known manner with the known tanning liquors composed of natural tanning substances or with natural 60 tanning baths and chromium compounds.

The present process reduces the time required for tanning to days and weeks, so that the present process is of very great economic importance, since it results in the production 65 of a good quality leather, which is equal to the so-called bark-tanned pit leather.

In addition, an entirely novel and improved chromium fibre may be obtained by means of a combined finishtanning with vegetable tan- 70 ning substances and chromium compounds.

The present process can also be used with advantage for preliminarily tanning pelts, since these latter can easily be depilated subsequently without any difficulty with known 75 liming agents, and worked up further to leather. This has the advantage that such preliminarily tanned pelts can be shipped a long distance without spoiling during trans- 80 port.

## Example

150 kgs. of thickened spent sulphite cellulose liquor, lignin sulphonic acid or tanning extracts are treated with about 20 kgs. hydrogen peroxide (30%) or also with suitable 85 solutions of compounds capable of liberating oxygen, such as perborates, persulphates and the like. Chlorine or bromine or both halogens are then added to this mixture in such 90 quantities or proportions that the reaction product absorbs about 6 to 10%. The quantity or proportions of chlorine or bromine can, however, be selected as desired, according to whether a weak or strong tanning effect is desired.

60 kgs. of the above reaction product are diluted with about 100 kgs. water and can then be used for the preliminary tanning of 100 pelts, hides or skins.

After the hides have been penetrated to a sufficient extent, they are finished-tanned with vegetable tanning baths or merely partially tanned with the latter and then finish 5 tanned with known chromium compounds, for instance with basic chromium sulphate solution.

It is evident that use may also be made of dilute spent sulphite cellulose liquor, and also 10 of dilute tanning extracts or mixtures thereof.

In that case it is merely necessary to take into consideration the quantity or proportions of the substance giving off oxygen and 15 the halogens.

I claim:—

1. A process of pre-tanning animal hides and pelts, comprising the step of pre-tanning the hides with a halogen reaction product obtained by bringing sulphite cellulose liquor 20 into reaction with hydrogen peroxide and then halogenating.

2. A process of pre-tanning animal hides and pelts, comprising the step of pre-tanning the hides with a halogen reaction product obtained by bringing sulphite cellulose liquor into reaction with an oxygen liberating substance of the class consisting of peroxides, 25 perborates and persulfates of alkali and then 30 halogenating.

3. A process of pre-tanning animal hides and pelts, comprising the step of pre-tanning the hides with a spent tanning liquor to which 35 has been added the halogenated reaction product obtained by acting upon sulphite cellulose liquor with a member of the class consisting of hydrogen peroxide, alkali peroxide, alkali 40 perborate and alkali persulfate and then halogenating.

4. A process of tanning animal hides and pelts, comprising the steps of pre-tanning the hides with a halogenated reaction product obtained by reacting upon sulphite cellulose liquor with a member of the class consisting 45 of hydrogen peroxide, alkali peroxide, alkali perborate and alkali persulfate and halogenating such reaction product, and then 50 finish-tanning the hides with a natural tanning substance.

5. As a new product, an animal hide which has been pre-tanned with a halogenated reaction product obtained by reacting upon sulphite cellulose waste liquor with a member of the class consisting of hydrogen peroxide, 55 alkali peroxide, alkali perborate and alkali persulfate and halogenating such reaction product.

6. As a new product, an animal hide which has been subjected to the respective steps of 60 pre-tanning and finish-tanning, the pre-tanning step consisting in wetting the hide with the halogenated reaction product obtained by reacting upon sulphite cellulose waste liquor with a member of the class consisting of hydrogen peroxide, alkali peroxide, alkali per- 65

borate and alkali persulfate and halogenating said reaction product, and the finish-tanning step consisting of wetting the pre-tanned hide with a natural tanning substance.

7. A new tanning composition of matter 70 comprising the halogenated reaction product of sulfite cellulose liquor and hydrogen peroxide.

In testimony whereof I have hereunto set my hand.

WILHELM SAILER.

80

85

90

95

100

105

110

115

120

125

130